

1  
2,984,556**FUEL COMPOSITION AND PROCESS FOR ITS  
MANUFACTURE****Samuel K. Talley, Berkeley, Calif., assignor to Shell Oil  
Company, a corporation of Delaware****No Drawing. Filed Mar. 19, 1954, Ser. No. 417,502****7 Claims. (Cl. 52—5)**

This invention is concerned with the improvement in the properties of ammonium nitrate and similar water-soluble crystalline oxidizing agents. More particularly, it is directed to a process for the preparation of an improved ammonium nitrate and to its use in fuel compositions.

The utilization of ammonium nitrate as an oxidizing agent and for other purposes is limited by a number of its properties, such as the low viscosity of the material in its melted state. A second shortcoming of ammonium nitrate is its change in volume at relatively low temperatures (e.g., at about 32° C.), at which point the volume of the solid material increases about 4%. Another difficulty encountered with ammonium nitrate is its tendency to cake during storage, apparently due to absorption of moisture. Finally, particularly where it is utilized as an oxidant in fuel compositions, its rate of decomposition and combustion are lower than sometimes desirable.

Ammonium nitrate (and other oxidizing agents such as potassium perchlorate or ammonium perchlorate) is an available oxidizing agent which may be used in conjunction with combustible substances for such purposes as rocket fuels, jet assisted take-off fuels, and the like. In such systems the combustible material is preferably intimately mixed with the oxidizing agent and the mixture ignited to produce the propelling action necessary for rockets or other similar missiles. It has been determined that the rate of burning of such fuel compositions is much lower than desired for many potential applications and it has been further determined that this low rate of burning may be due to the adverse physical properties of both the combustible substance phase and the ammonium nitrate phase especially at or above their melt temperatures. Photographic studies have shown that rocket fuel compositions comprising asphalt and ammonium nitrate mixtures burn at a slow rate or actually cause snuffing of the flame at the burning phase, due to the low viscosity of one or the other phase which covers the burning face and thus snuffs out the flame. A co-pending United States application by Samuel K. Talley, Serial No. 406,902, filed January 28, 1954, relates to the improvement in the properties of the combustible material (which is combined with ammonium nitrate and the like) whereby the viscosity and other properties of the combustible substance at or above its melting point is improved. The properties of the plastic combustible substance may be greatly altered by the presence of compatible or incompatible plasticizers therefor, or combinations of such types of plasticizers, and further by the incorporation of high temperature thickening agents. It has been found that combustible substances such as bituminous materials may be improved greatly with respect to their response to temperature change and more particularly in their viscosity properties at elevated temperatures.

While the properties of the plastic combustible materials thus can be improved markedly, this leaves much to be desired with respect to the burning rates and other burning qualities of such compositions when combined

with ammonium nitrate or the like. While the properties of the phase containing the combustible material are improved, it would appear to be necessary to improve the properties of ammonium nitrate at or above its melt temperature so as to obtain optimum burning properties.

It is an object of the present invention to improve the properties of ammonium nitrate and/or other oxidizing agents. It is a particular object of this invention to improve the properties of ammonium nitrate at or above its melt temperature. It is a further object of this invention to improve the burning properties of fuel compositions containing ammonium nitrate. It is another object of the invention to depress or alter the phase change temperature of ammonium nitrate. Other objects will 15 become apparent during their following discussion.

Now, in accordance with this invention, it has been found that the thickening effect of high temperature thickening agents upon ammonium nitrate is substantially increased by combining the thickening agent with an

20 aqueous solution of the nitrate prior to dehydrating the latter (rather than by dry mixing). Still in accordance with this invention, further improvements in the properties of ammonium nitrate may be made by the further modification of the substance with potassium nitrate and/or ammonium dichromate. Again in accordance with this invention, it has been found that ammonium nitrate compositions modified by the process outlined above provide especially desirable properties for their incorporation in fuel compositions and especially in rocket fuel 30 compositions.

The properties of ammonium nitrate have been modified by the dry mixing of nitrate with various other substances such as Prussian blue and the like. However it has been ascertained that the improvement in ammonium 35 nitrate caused by such method of incorporation is only of a minor order and that the improvement is not sufficient to be satisfactory. The present process comprises addition of Prussian blue and other high temperature thickening agents outlined hereinafter to ammonium nitrate (or inorganic perchlorates) while the latter is in aqueous solution and thereafter dehydrating the mixture thus formed. The incorporation of the modifying substances by this method produces ammonium nitrate having properties, especially at its melt or burning temperatures, substantially better than those obtained by the dry mixing 45 of the separate ingredients.

In carrying out the process of the present invention, it is necessary to have only sufficient water present to form a liquid phase into which the modifying ingredients are 50 mixed or in which the ingredients are formed. At elevated temperatures in the order of 200° F. and above, very small percentages of water in the order of 2-5% of water cause the formation of liquid solutions with ammonium nitrate. Consequently, the ammonium nitrate 55 may be dry at room temperature, or apparently so, but may contain sufficient water to be in a liquid state at an elevated temperature and suitable for use in the present process. However, the process is not confined to the use of systems in which such small proportions of water 60 exist. On the contrary, it is possible to use any greater amount of water desired, for example, 30-70% of water based on the total of water and ammonium nitrate. Under these conditions, of course, the temperature at which liquid solutions exist is of a considerably lower 65 order, such as between room temperature and 200° F. The dehydration may be carried out by any desired means. If minimum particle size of the dried material is desired, the solution of the water-soluble ingredients 70 may be emulsified with a water-immiscible (preferably volatile) liquid, using 1-5% based on the solids, of an emulsifying agent capable of forming a water-in-oil type

of emulsion; dehydrating the emulsion and removing the water-immiscible liquid.

The modifying ingredients which may be employed in the present process for the purpose of increasing the viscosity of the molten ammonium nitrate include especially amorphous inorganic colloidal substances, clay materials as defined hereinafter, carbon blacks and Prussian blue.

The clay materials useful in the present process and for the preparation of the novel compositions more fully described hereinafter include especially high base exchange clays, onium-clays (reaction products of natural clays with onium compounds) and natural clays bearing hydrophobic substances absorbed on their surfaces. The naturally occurring materials are mainly those of clay-like nature and preferably comprise the swelling type of bentonite clays. While the swelling type of clays are preferred, the non-swelling types such as Georgia kaolinite also may be used. Optimum compositions may be obtained by the use of magnesium montmorillonite, such as hectorite. The Wyoming bentonite ordinarily regarded as aluminum montmorillonite, also is highly effective.

Synthetic materials may be prepared having properties suitable for use in the present process and similar to the naturally occurring materials insofar as their present function is concerned. Since they are so closely similar to the naturally occurring clays, they are for the present specification and claims to be regarded as included in the term "clay materials." These synthetic materials are also called synthetic zeolites. The purposes for preparing and using synthetic clay-like materials are to avoid the presence of non-colloidal impurities if this is desirable, or at least to have under close control the exact composition of the colloid, e.g., the relative proportions of silica, alumina and sodium oxide or other oxide which may be varied within wide ratios. The preferred variety of synthetic zeolite comprises alumina-silicate which may be regarded as compounds of alumina and silica containing varying ratios of sodium oxide.

Onium clays are normally prepared by reaction of an onium compound such as a quaternary ammonium salt with a clay having a relatively high base exchange capacity, generally between about 25 and about 100 milliequivalents of exchangeable base per hundred grams of clay. The onium compounds such as those described hereinafter are of such a type and are employed in such a proportion as to provide an onium clay reaction product swelling at least eight-fold in nitrobenzene. Compositions of this character are described in the Hauser patent, U.S. 2,531,427.

Onium compounds which may be utilized in the formation of onium clays include, for example, naphthylammonium chloride, dicyclohexylammonium bromide, lauryldimethylammonium chloride, tetraethanolammonium bromide, octadecylammonium iodide, and laurylphosphonium bromide as well as dimethyldicetylammonium bromide.

In addition to the naturally occurring (or synthetic) clay-like materials and their onium derivatives, another variety of high temperature thickener may be prepared by simple adsorption of a hydrophobic agent on the surfaces of the clay without any substantial degree of chemical reaction therewith. In the preparation of hydrophobic clay materials of this class, primary, secondary or tertiary alkyl amines and other aliphatic amines are preferred. These include such amines as dodecyl amine, hexadecyl amine, octadecyl amine and mixtures thereof. Preferably, the amines should contain at least ten carbon atoms and still more preferably at least ten carbon atoms in a single aliphatic hydrocarbon chain. Other suitable means useful in these compositions include cyclic amines such as naphthylamine, heterocyclic amines such as pyridine and pyrimidine derivatives and tetrahydro pyrimidines, as well as, polyamines and amidoamines.

The carbon blacks which may be employed in improv-

ing the properties of ammonium nitrate include such materials as furnace blacks and channel blacks, the former being characterized by generally smaller surface areas and larger particle sizes than the latter. Furnace black surface areas range from about 3 to about 100 square meters per gram, equivalent to about 0.4 to 0.5 micron average particle diameter. On the other hand, channel blacks range from about 100 to about 200 square meters per gram, equivalent to 0.2-0.4 micron average particle diameter. These blacks are known in the trade under other names, such as channel black, acetylene black lamp black and thermal black. Mixtures of the blacks may be obtained in order to modify the thickening properties of molten ammonium nitrate.

Amorphous inorganic colloidal materials suitable for the present purpose include silica, alumina, magnesia, vanadium oxide, and ferric oxide, as well as the corresponding hydroxides (including lime), alkaline earth carbonates, such as calcium carbonate, etc. Preferably these inorganic colloidal substances are in the form of highly porous materials typified by (but not exclusively restricted to) aerogels and the like. Preferably the amorphous colloids have surface areas in the order of 100 square meters per gram or higher. They may be prepared by a number of well-known methods, such as the burning of silicon tetrahalide to form finely divided silicon oxide, or may be formed by solvent replacement, such as the replacement of water from an inorganic hydrogel with alcohol and subsequent removal of the alcohol by heating the alcogel in an autoclave to a temperature above the critical temperature of the alcohol and thereafter releasing the pressure so as to form a highly porous gel sometimes referred to as an aerogel. Another material suitable for the present purpose is Prussian blue.

Modification of ammonium nitrate with such materials as 5% by weight of jewelers' rouge or calcium silicate (or other modifiers such as those described above) by dry mixing of the ingredients resulted in no apparent advantage, since the mixture, upon melting was very fluid. However, addition of the same materials to a 50% aqueous solution of ammonium nitrate, followed by dehydration, resulted in mixtures which were pasty in their melted state. Furthermore, the latter compositions did not readily separate from asphalt at the melt temperatures, when such compositions were being burned.

One of the disadvantages of ammonium nitrate comprises its volume change at various temperatures. An important phase change temperature is about 32° C., a temperature commonly encountered in the storage and use of shaped charges such as rocket fuels. This volumetric change is disadvantageous due to the fact that it causes cracking of the charge and thereby results in uneven burning thereof. Certain materials may be added to ammonium nitrate to minimize or alter this phase change. Potassium nitrate may be added for the purpose of increasing the temperature at which the volumetric change occurs to a limited extent. It has been found, in accordance with one phase of this invention, that the addition of the above defined thickening agents also has a retarding effect upon the phase change and may show a synergistic effect when combined with potassium nitrate. Table I below illustrates these properties.

Table I

|    | Additive                                 | Volume Change Temperature, °C. |
|----|------------------------------------------|--------------------------------|
| 65 | None                                     | 32                             |
| 70 | 5% Prussian blue                         | 42                             |
|    | 4.3% Prussian blue+5.3% KNO <sub>3</sub> | 48                             |
|    | 5% Silica                                | 42                             |
|    | 5% Alumina                               | 38                             |

The addition of Prussian blue increased the volume change temperature by 10 degrees. Combination of Prussian

blue with potassium nitrate caused a 16 degree rise in the volume change temperature while silica and alumina caused phase change temperatures of 10 and 6° C., respectively. These additives were incorporated in ammonium nitrate by the wet process described hereinbefore.

In addition to correction of the viscosity of molten ammonium nitrate, it has been found that the additives, when incorporated with the nitrate by the wet process described hereinbefore, causes catalysis of the oxidizing action of the nitrate. Not only is oxidation catalysed, but the stiffening agents appear to act as synergists when combined with other catalysts, such as ammonium dichromate. This will become apparent in the burning tests to be described hereinafter.

As pointed out hereinbefore, one of the principal uses of modified ammonium nitrate prepared as described above is in the compounding of fuels and particularly of guided missile or rocket fuels. Broadly, the class of fuels considered here are plastic solids comprising a combustible material intimately commingled with an oxidizing agent and providing the propellant power for rockets and the like to be used in missiles or for jet aircraft takeoff or for added power during aircraft flight. The principal combustible materials considered for use in these plastic solid fuels include bituminous substances, organic polymers, including resins or rubbers, and cellulose compounds, including cellulose ethers or esters, such as ethyl cellulose, cellulose acetate and cellulose nitrate. These solid combustible materials perform the dual function of fuels and plastic materials capable of being molded together with the oxidizing agent into a plastic solid fuel charge. Therefore, an important aspect of the present invention comprises the utilization of the modified ammonium nitrates (or other oxidizing agents, such as modified ammonium perchlorate) in plastic solid fuels of this type.

The bituminous substances which may be employed in the subject plastic solid fuels comprise for the most part those of petroleum origin or derived from coal tar or coal tar pitch. The essential requirement for the compositions under consideration is that the bituminous substance have an ASTM penetration at 77° F. (five seconds, 100 gram load) less than about 20 dmm. and preferably less than 10 dmm. This is then plasticized to yield a binder fuel having an ASTM penetration of about 150-250 dmm. at 77° F. The bituminous materials also should have an ASTM ring and ball softening point between about 150 and about 300° F., and preferably between 175 and 225° F. Suitable materials may be prepared by the use of one or more asphaltic or coal tar components and may be either blown or unblown petroleum products.

An asphalt suitable for the present purpose may be prepared, for example, by air blowing of either distilled or residual petroleum fractions. For example, short residue, heavy bulk distillates, lubricating oil extracts or bright stocks may be blown to suitable asphaltic compositions having a desired penetration range. Preferably, the starting materials contain only a minor amount of aromatic fractions, and short residues obtained from the West Texas fields are preferred. It is still more preferred that asphalts are employed having softening points above about 285° F. and are the dewaxed residue of a mixed base crude. In addition to the asphalts and coal tar pitches suitable for use in these compositions, asphaltites, such as gilsonite and grahamite may be employed either as the sole bituminous substance or in combination with one or more of the above materials.

As discussed in the co-pending application of Samuel K. Talley, Serial No. 406,902, of which this case is in part a continuation-in-part, one of the serious shortcomings of a number of these plastic fuels comprises their highly fluid character when in the molten state. Accordingly, it was found that certain stiffening agents could be employed to overcome or minimize this de-

iciency and comprise the general class of stiffening agents described hereinbefore and which are now being added to the ammonium nitrate phase.

It has been found that the addition of the stiffening agent to one phase only is not sufficient to cause stiffening of both phases, but that the stiffening agents are most effective if separately incorporated in each phase prior to combination of the two phases in the final assembly of the fuel composition.

Furthermore, certain of the fuels, such as the bituminous materials described above, exhibit disadvantageous properties with respect to change in viscosity and consistency with change in temperature. It has been found that these properties can be radically altered by modification of the bituminous material with certain esters or mineral lubricating oils.

The esters are fully described in the co-pending parent application and generally comprise phosphorus esters (particularly, normally liquid aliphatic esters of phosphorus; organic silicate esters and aliphatic esters of polycarboxylic acids). Typical esters include the trialkyl phosphates, such as trioctyl phosphate, trihexyl phosphate, tridecyl phosphate and other phosphates containing a total of at least eighteen carbon atoms per molecule and preferably between about 20 and 32 carbon atoms per molecule. The corresponding phosphinates and phosphonates may be employed, such as di(2-ethylhexyl)hexane phosphonate. Silicate esters include alkyl, aryl, aralkyl and alkylaryl esters of silicic acid. Typical members of these classes include tetra(2-ethylhexyl)silicate and tetracresyl silicate. Suitable dicarboxylic esters include di(2-ethylhexyl)sebacate and other typical aliphatic esters, such as those disclosed in U.S. Patent 2,481,372.

As the parent application of Samuel K. Talley, referred to above, shows, a combination of high temperature thickening agents and the plasticizing materials produces a particularly beneficial type of bituminous composition. This is especially suitable for its low response to temperature changes such as may be required in the use of the bituminous compositions as fuels in combination with the modified nitrates (or perchlorates). Consequently, an important feature of this invention comprises the combination of the modified ammonium nitrates prepared by the wet process described hereinbefore combined with bituminous compositions containing both a high temperature thickening agent and a plasticizing material of the class described. Preferred compositions containing these two modified phases are as follows:

Table II

|                                              | Percent by Weight of the Phase | Percent by Weight of Total Composition |
|----------------------------------------------|--------------------------------|----------------------------------------|
| Ammonium nitrate phase:                      |                                |                                        |
| Ammonium nitrate .....                       | 96-80                          |                                        |
| Potassium nitrate .....                      | 2-10                           |                                        |
| Thickener (incorporated by wet method) ..... | 2-10                           | 60-90                                  |
| Bituminous fuel phase:                       |                                |                                        |
| Bitumen .....                                | 79-25                          |                                        |
| Plasticizer .....                            | 20-65                          |                                        |
| Thickener .....                              | 1-10                           | 40-10                                  |

The practical significance of the modification of both the ammonium nitrate phase and the plastic fuel phase substantially as described above is readily determined in the relative burning rates of compositions omitting or containing the modifying substances as demonstrated by the data given hereinafter. Burning strands having a quarter inch cross-section were compounded by intimately mixing the bituminous fuel phase and the ammonium nitrate oxidant phase and burning them in a nitrogen or inert atmosphere at one thousand pounds per square inch gauge pressure. If such strands are prepared by mixing fifteen parts by weight of a hard blown asphalt with 85 parts by weight of finely ground ammonium nitrate, the

resulting flame is quickly snuffed out due to the melting and separation of the components which retard or even prevent the ammonium nitrate from contacting the burning phase. Modification of the asphalt with 1% by weight of the total composition of the reaction product of bentonite and dicetyltrimethylammonium chloride (Benton 34 trade name) resulted in a burning rate of 0.06 inch per second. The use of 5%, based on the total composition, of a catalyst (ammonium dicromate) mixed with the ammonium nitrate phase and of 1% (based on the total composition) of the same onium clay dispersed in the asphalt phase, resulted in a burning rate substantially twice that of the second sample, namely, 0.127 inch per second. However, by incorporation of a thickening agent in the ammonium nitrate phase by the wet method described hereinbefore, the burning rate was increased to nearly triple that of the second sample described above. Wet mixing of potassium nitrate with ammonium nitrate did not result in any burning rate advantage. The following table gives typical results of such experiments:

- 8
3. A fuel composition according to claim 1 wherein potassium nitrate also is dispersed throughout the ammonium nitrate phase.
  4. A fuel composition according to claim 1 wherein the asphalt phase comprises an oxidized asphalt material.
  5. A fuel composition comprising predominantly 10-40% by weight of an asphalt phase having colloidally dispersed therethrough a clay material and a separate phase commingled therewith comprising 60-90% by weight of ammonium nitrate having dispersed therethrough a thickening agent selected from the group consisting of colloidal silica gel, clay, ammonium clays capable of swelling at least 8-fold in nitrobenzene, clays bearing hydrophobic amines adsorbed on the surfaces thereof, carbon blacks and Prussian blue; the proportion of thickening agents being sufficient to substantially thicken both phases when they are melted, said agent constituting 1-10% by weight of the asphalt phase and 2-10% by weight of the ammonium nitrate phase.
  10. 15. 20. 6. In a method for the production of improved fuel

| Sample | Amount, Percent w.     | Component                                                | Wet Mix Avg. Burning Rate, in./sec. | Dry Mix Burning Rate |
|--------|------------------------|----------------------------------------------------------|-------------------------------------|----------------------|
| A      | 14                     | Asphalt C                                                | .127                                | -----                |
|        | 1                      | Bentonite 34                                             |                                     |                      |
|        | 80                     | Ammonium nitrate, 3X ground                              |                                     |                      |
|        | 5                      | Ammonium dichromate, ground                              |                                     |                      |
| B      | 14                     | Asphalt C                                                | .151                                | .116                 |
|        | 1                      | Bentonite 34                                             |                                     |                      |
|        | 85                     | { 85. ammonium nitrate<br>4.3 Prussian blue } 3X ground  |                                     |                      |
|        | 10.3 potassium nitrate |                                                          |                                     |                      |
| C      | 14                     | Asphalt C                                                | .208                                | -----                |
|        | 1                      | Bentonite 34                                             |                                     |                      |
|        | 80                     | { 85. ammonium nitrate<br>4.3 Prussian blue } 3X ground  |                                     |                      |
|        | 10.3 potassium nitrate |                                                          |                                     |                      |
| D      | 5                      | Ammonium dichromate, ground                              | .172                                | -----                |
|        | 14                     | Asphalt C                                                |                                     |                      |
|        | 1                      | Bentonite 34                                             |                                     |                      |
|        | 91.0 ammonium nitrate  | { 91.0 ammonium nitrate<br>4.5 furnace black } 3X ground |                                     |                      |
| E      | 85                     | 4.5 potassium nitrate                                    | .188                                | -----                |
|        | 14                     | Asphalt C                                                |                                     |                      |
|        | 1                      | Bentonite 34                                             |                                     |                      |
|        | 85                     | { 91.0 ammonium nitrate<br>4.5 furnace black } 3X ground |                                     |                      |
| F      | 5                      | 4.5 potassium nitrate                                    | .101                                | .081                 |
|        | 14                     | Ammonium dichromate, ground                              |                                     |                      |
|        | 1                      | Asphalt C                                                |                                     |                      |
|        | 95 ammonium nitrate    | { 95 ammonium nitrate<br>5 Prussian blue }               |                                     |                      |
| G      | 85                     | Asphalt C                                                | .081                                | -----                |
|        | 1                      | Bentonite 34                                             |                                     |                      |
| G      | 85                     | { 95 ammonium nitrate<br>10 potassium nitrate }          |                                     |                      |

Asphalt C, used in the above rocket fuels, comprised 64% by weight of a commercial blown asphalt (penetration=19 dmm. at 77° F.) combined with 36% by weight of a West Texas mineral lubricating oil having a viscosity of about 100 SUS at 100° F. and a viscosity index of about 90.

I claim as my invention:

1. A fuel composition consisting essentially of an asphalt phase and a separate ammonium nitrate phase commingled therewith, each phase having intimately dispersed therethrough a thickening agent of the group consisting of colloidal silica gel, clay, ammonium clays capable of swelling at least 8-fold in nitrobenzene, clays bearing hydrophobic amines adsorbed on the surfaces thereof, carbon blacks and Prussian blue, the amount of thickening agent present in each phase being at least sufficient to substantially thicken the phases when they are melted, said agent constituting 1-10% by weight of the asphalt phase and 2-10% by weight of the ammonium nitrate phase.

2. A fuel composition according to claim 1, wherein ammonium dichromate also is dispersed throughout the nitrate phase.

55. 60. 65. 70. compositions, the steps comprising combining ammonium nitrate in aqueous solution with a thickening agent and thereafter dehydrating the combined components whereby a thickened ammonium nitrate phase is formed; combining an asphalt with a thickening agent whereby a thickened asphalt phase is formed; and milling 60-90 percent by weight, based on the total composition, of the thickened ammonium nitrate phase with 40-10 percent by weight, based on the total composition, of the thickened asphalt phase whereby a fuel composition is formed; the thickening agent present in each of the phases being selected from the group consisting of colloidal silica gel, clay, ammonium clays capable of swelling at least 8-fold in nitrobenzene, clays having a hydrophobic amine adsorbed on the surfaces thereof, carbon blacks and Prussian blue, the proportion of thickener being 2-10% by weight in the ammonium nitrate phase and 1-10 percent by weight in the asphalt phase.

75. 7. A fuel composition comprising an asphalt phase and a separate ammonium nitrate phase commingled therewith, the asphalt phase having dispersed therethrough 2-10% by weight of an ammonium clay capable of swelling at least 8-fold in nitrobenzene, and the ammonium

nitrate phase having 1-10% by weight of Prussian blue dispersed therethrough.

References Cited in the file of this patent

UNITED STATES PATENTS

1,021,882 O'Brien ----- Apr. 2, 1912  
2,159,234 Taylor ----- May 23, 1939

5

2,434,872  
2,531,427  
2,661,301

Taylor et al. ----- Jan. 20, 1948  
Hauser ----- Nov. 28, 1950  
Capell ----- Dec. 1, 1953

FOREIGN PATENTS

Great Britain ----- 1897  
Great Britain ----- July 25, 1951